

## UNITED STATES PATENT OFFICE

2,448,462

## CORROSION RESISTANT STEEL AND EQUIPMENT

Louis Secondo Renzoni, Port Colborne, Ontario, Canada, assignor to International Nickel Company, Inc., New York, N. Y., a corporation of Delaware

No Drawing. Application March 20, 1946, Serial No. 655,893. In Canada February 12, 1946

11 Claims. (Cl. 75—128)

1

The present invention relates to alloy steels, and chemical equipment made therefrom, which are highly resistant to very corrosive acidic chloride-bearing solutions, particularly sulfate-chloride and all-chloride solutions.

Numerous alloy steels have been proposed to resist various corrosive solutions but none, as far as is known, had satisfactory resistance to highly corrosive acidic chloride-bearing solutions, such as aqueous sulfate-chloride and all-chloride solutions. As a result, the art heretofore relied upon various non-metallic materials in constructing or coating certain commercial chemical equipment or apparatus exposed in use to contact with such acidic chloride solutions. For example, mastic-lined concrete tanks can be employed to handle acidic sulfate-chloride or all-chloride aqueous solutions, e. g., in the electrolytic refining of nickel with a sulfate-chloride electrolyte such as described in my co-pending United States application, Serial No. 472,471, now U. S. Patent No. 2,394,874. However, the chloride-bearing solutions have to be conveyed into and out of containers, tanks, vats, etc., by means of pumps and through valves, pipes, conduits and the like, for which uses non-metallic materials are not suitable. A need existed for an alloy steel highly resistant to corrosive acidic chloride-bearing solutions, particularly impure chloride solutions which are very corrosive, which steel could be used for the manufacture of pump castings, valve castings, pipes, containers and like chemical equipment or apparatus. Although many attempts were made to provide alloy steels highly resistant to corrosive aqueous acidic chloride-bearing solutions, none, as far as I am aware, was successful when carried into commercial use.

I have discovered an alloy steel highly resistant to corrosive aqueous acidic chloride-bearing solutions, including the very corrosive impure sulfate-chloride and all-chloride solutions, having a critical composition within a narrow range and containing nickel, chromium and molybdenum.

It is an object of the present invention to provide an alloy steel, and articles made therefrom, highly resistant to aqueous acidic chloride-bearing solutions.

It is another object of the invention to provide an alloy steel highly resistant to extremely corrosive impure sulfate-chloride and all-chloride

2

acidic solutions, and particularly suitable for making chemical equipment such as pump castings, valve castings, cast pipes, containers and the like.

5 It is a further object of the present invention to provide chemical equipment for handling corrosive aqueous acidic chloride-bearing solutions, which equipment is made of an improved alloy steel highly resistant to such solutions.

10 Other objects of the invention will become apparent to those skilled in the art from the following description.

The alloy steel provided by the present invention is highly resistant to very corrosive aqueous 15 chloride-bearing solutions, including sulfate-chloride and all-chloride solutions, and comprises 21% to 23% nickel, 21% to 22% chromium, 5% to 6% molybdenum, not more than about 0.15% carbon, preferably not more than 0.12% carbon, 20 and the balance substantially all iron. It is desirable that the chromium content not exceed the nickel and that the nickel content increase with increasing chromium content within the aforementioned ranges. Preferably, the nickel content is maintained within the range of 22% to 23%. It is essential that the foregoing controlled 25 compositions be employed as a substantial departure from said ranges results in failure to achieve the desired results, including the high corrosion 30 resistance provided by the alloy steels having compositions within the aforementioned ranges. The alloy steels having the foregoing composition are characterized by a completely austenitic structure. It is essential that the steels of the 35 present invention be devoid of a second phase such as the well-known sigma phase which is often present in high-chromium iron-base compositions. The mere absence in an austenitic alloy steel of a second phase such as the sigma 40 phase does not in itself mean that the alloy steel will be corrosion resistant to the aforementioned acidic aqueous chloride-bearing solutions, including impure sulfate-chloride and all-chloride solutions. It is also essential in order to obtain high 45 corrosion resistance to such acidic aqueous chloride solutions that the completely austenitic composition be maintained within the range of compositions set forth hereinbefore. A feature of said composition is the critical proportioning of the nickel content to the chromium and molyb-

denum contents. Carbon is not an essential element and is tolerated mainly because it is commercially impracticable to produce the metal composition without some carbon being present. It is preferred to maintain the carbon content as low as commercially feasible. Because some carbon is usually present, the compositions have been referred to as a steel. The present invention does not exclude the presence of the usual small amounts, say up to a total of about 1% or 1.5%, of other elements which are commonly present in or added to steels, especially of the austenitic type, as a result of good steel-making practice or for known purposes. Illustrative examples include the normal content of sulfur, phosphorus, manganese, silicon, copper, titanium, columbium, etc. As silicon and manganese strongly promote the formation of the sigma phase, it is preferable that the amounts of these elements be held to a minimum or even avoided entirely whenever practicable. Titanium or columbium are frequently employed to fix carbides and may be present, especially if the carbon content is sufficiently high to promote excessive carbide precipitation.

The invention contemplates corrosion-resistant articles, including chemical equipment, particularly those made of cast alloys, such as pump castings, valve castings, cast pipes, containers and the like, made of the special compositions described herein.

An illustrative example of an alloy steel contemplated by the invention and having high resistance to corrosion by acidic aqueous chloride solutions, particularly the impure sulfate-chloride solutions such as the impure anolyte or electrolyte used in the process described in my co-pending application, Serial No. 472,471, now U. S. Patent No. 2,394,874, has the following composition:

|            | Per cent |
|------------|----------|
| Nickel     | 22.8     |
| Chromium   | 21.1     |
| Molybdenum | 5.4      |
| Carbon     | 0.11     |
| Iron       | Balance  |

Pumps and conduits made of the foregoing composition have given satisfactory results when used in the process of my above-mentioned application to convey the impure electrolyte from the holding tank to the unit for the removal of impurities such as iron, arsenic and lead. Compositions within the ranges set forth hereinbefore have also given good results in the carrying out of the process described in the aforementioned patent application when used as pipes, pumps, valves, etc., for conducting and treating the electrolyte from the electrorefining tanks to tank No. 15 in Fig. 7 of my co-pending patent application, Serial No. 472,471, now U. S. Patent No. 2,394,874.

In order to assure the corrosion resistance contemplated by the invention, it is highly desirable that the alloys be in the heat-treated condition resulting from an annealing treatment followed by a rapid cooling, e. g., a water quench. Such a heat treatment is particularly desirable when carbon is present in amounts sufficient to result in the precipitation of carbides at the grain boundaries. The heat treatment also assures the absence of a second phase such as the sigma phase. A suitable annealing treatment comprises holding the alloy or the casting at a temperature of about 2150° to 2250° F. for periods of about 15 minutes to one hour depending on

the cross-sectional size followed immediately by a water quench.

In order that those skilled in the art may have a better understanding of the invention and a better appreciation of the critical nature of the composition and of the improved corrosion resistance obtained by the present invention, the corrosion resistant properties of compositions contemplated by the invention are compared with other compositions in the tables set forth hereinafter. Tables I and II give the percentage of carbon and various alloying elements present, in addition to iron, in the compositions. All compositions, i. e., No. 1 to No. 17, were given the same heat treatment described hereinbefore, i. e., annealed at about 2250° F. followed immediately by a water quench.

Table I

| Steel No. | Composition |             |             |            | Structure              |
|-----------|-------------|-------------|-------------|------------|------------------------|
|           | Per cent Ni | Per cent Cr | Per cent Mo | Per cent C |                        |
| 25        |             |             |             |            |                        |
| 1         | 22.0        | 21.0        | 5.0         | 0.12       | All austenite.         |
| 2         | 21.0        | 22.0        | 5.5         | 0.12       | Do.                    |
| 3         | 21.0        | 23.0        | 5.5         | 0.12       | Austenite+sigma phase. |
| 4         | 21.0        | 22.0        | 6.5         | 0.10       | Do.                    |
| 5         | 22.0        | 21.0        | 6.9         | 0.09       | Do.                    |
| 6         | 20.2        | 21.7        | 3.0         | 0.12       | All austenite.         |
| 7         | 25.0        | 20.0        | 5.1         | 0.11       | Do.                    |
| 8         | 30.0        | 24.0        | 5.5         | 0.10       | Austenite+sigma phase. |
| 9         | 35.0        | 25.0        | 5.0         | 0.20       | Do.                    |
| 10        | 12.0        | 20.0        | 4.0         | 0.10       | Do.                    |
| 11        | 12.0        | 20.0        | 5.0         | 0.10       | Do.                    |
| 12        | 12.0        | 20.0        | 8.0         | 0.10       | Do.                    |

Table II

| Steel No. | Composition |             |             |                    |             |             | Structure      |
|-----------|-------------|-------------|-------------|--------------------|-------------|-------------|----------------|
|           | Per cent Ni | Per cent Cr | Per cent Mo | Per cent C         | Per cent Cu | Per cent Si |                |
| 40        |             |             |             |                    |             |             |                |
| 13        | 22          | 19          | 3.5         | 0.07               | 1.0         | 1.25        | All austenite. |
| 14        | 22          | 19          | 3.5         | 0.07               | 1.0         | -----       | Do.            |
| 15        | 24          | 22          | 3.0         | 0.07               | 1.75        | 3.25        | Do.            |
| 45        | 30          | 20          | 3.0         | 0.07               | 5.0         | -----       | Do.            |
| 16        | 35          | 15          | 3.0         | n. d. <sup>1</sup> | -----       | -----       | Do.            |
| 17        |             |             |             |                    |             |             |                |

<sup>1</sup> Not determined; estimated between 0.2% and 0.3% carbon.

50 Steels No. 1 and No. 2 are properly proportioned in accordance with the present invention. Steels No. 3 to No. 17 have compositions outside the critical compositions contemplated by the present invention and are included for comparative purposes. Steels No. 1 to No. 17 were all subjected under similar conditions to tests to ascertain their corrosion resistance. Because cast surfaces were found to be less resistant to attack than polished surfaces, the corrosion tests were conducted on as cast surfaces to more severely test the corrosion resistance of the steels. All steels were subjected to corrosion tests in a fully aerated impure sulfate-chloride acidic aqueous solution containing about 45 grams per liter of nickel, 0.25 gram per liter of copper, 0.1 gram per liter of iron, 30 grams per liter of sodium ion, 30 grams per liter of chloride ion, 95 grams per liter of sulfate ion, and 20 grams per liter of boric acid, and having a pH of about 3. These steels were moved through the solution at a rate of about 250 feet per minute for the same interval of time. The solution was maintained at a temperature of 150° to 155° F. The corrosion rate in milligrams per square decimeter per day (M. D. D.) was determined and the presence or absence of pitting noted on all

steels. The results of the tests are summarized in the following Table III.

Table III

| Steel No. | Corrosion Rate (M. D. D.) | Pitting |
|-----------|---------------------------|---------|
| 1         | 0 to 5                    | no.     |
| 2         | 0 to 5                    | no.     |
| 3         | 500                       | yes.    |
| 4         | 500                       | yes.    |
| 5         | 200                       | yes.    |
| 6         | 3,000                     | yes.    |
| 7         | 1,200                     | yes.    |
| 8         | 500                       | yes.    |
| 9         | 2,000                     | yes.    |
| 10        | 275                       | yes.    |
| 11        | 300                       | yes.    |
| 12        | 300                       | yes.    |
| 13        | 500                       | yes.    |
| 14        | 600                       | yes.    |
| 15        | 1,300                     | yes.    |
| 16        | 500                       | yes.    |
| 17        | 2,100                     | yes.    |

It will be observed from Table III that only the compositions made in accordance with the present invention, i. e., steels No. 1 and No. 2, had a low corrosion rate and did not exhibit pitting. All the other compositions, even those having compositions only slightly outside the range contemplated by the invention, had very much poorer resistance to corrosion, as evidenced by the high corrosion rate and by pitting. In general, the steels contemplated by the present invention and articles made therefrom exhibit, under the aforementioned test conditions, corrosion rates which usually do not exceed about 15 to 20 M. D. D.

Examples of other electrolytes in which the compositions contemplated by the invention exhibited satisfactory corrosion resistance include impure acidic nickel-containing sulfate-chloride or all-chloride aqueous solutions aerated to saturation, having a pH of 4.7, a temperature of 130° F. and containing 0.25 gram per liter of copper and 0.06 gram per liter of iron; acidic nickel-containing sulfate-chloride or all-chloride aqueous solutions having under slightly reducing conditions a pH of 4.8, a temperature of 140° F. and containing 0.15 gram per liter of copper and 0.0003 gram per liter of iron; acidic nickel-containing sulfate-chloride or all-chloride aqueous solutions (under slightly reducing conditions) having a pH of 5.3, a temperature of 150° F. and containing 0.005 gram per liter of copper and 0.0005 gram per liter of iron; etc.

It will be appreciated that the consistent production of steels within the range of compositions contemplated by the invention requires strict control of the composition during the production of the steel in order that it fall within the specified ranges. This is particularly true of the chromium content. Allowance must be made for any losses, particularly of chromium, during the melting process, and an excess of the element, e. g., chromium, must be added to compensate for any loss under the particular conditions. I have found it preferably to avoid the use of chromium-bearing scrap in the charge as the use of scrap renders the control of the chromium content more difficult and less predictable. The avoidance of any scrap is advantageous in maintaining the content of impurities at a minimum.

As noted hereinbefore, the present invention is particularly suitable for the production of cast chemical equipment subjected in use to contact with impure sulfate-chloride or all-chloride aqueous solutions, including electrolytes. Such solutions include the impure electrolytes em-

ployed in the process described in my aforementioned application. The impure solutions exhibit, in general, more severe corrosive action than pure solutions. Thus, arsenic and/or lead each in amounts of 0.0002 gram per liter or more and copper and/or iron each in amounts of 0.0005 gram per liter or more are considered to render solutions impure. Sulfate-chloride and all-chloride acidic solutions containing nickel and/or cobalt are much more corrosive when they also contain such impurities as iron and/or copper. Iron is particularly corrosive when present in amounts of about 0.005 gram per liter or more, especially when the iron is present in both the oxidized (ferric) and reduced (ferrous) forms as, for instance, during the oxidation of ferrous to ferric iron in chloride-bearing acidic aqueous solutions. Copper present in amounts of about 0.02 gram per liter or more renders chloride-bearing aqueous acidic solutions much more corrosive. The corrosive action due to the presence of copper is particularly severe when both the reduced (cuprous) and oxidized (cupric) forms are present as is the case during aeration of impure electrolytes to oxidize the iron. Aeration of acidic chloride-bearing nickel solutions has been found to accelerate considerably corrosion in such solutions, and the compositions of the present invention exhibit excellent corrosion resistance in aerated solutions, including aerated impure solutions. Excellent corrosion resistance has been obtained by the present invention in acidic chloride - bearing nickel - containing aqueous solutions having a pH between about 2 and about 5.5.

Excellent corrosion resistance is obtained by the present invention in the corrosive chloride-bearing acidic aqueous solutions containing at least about 2 grams per liter of chloride ions. With increasing chloride ion concentration, the corrosiveness will increase but the corrosive action reaches a maximum and generally remains substantially the same regardless of further increases in chloride concentration whether in a sulfate-chloride solution or an all-chloride solution. Thus, the maximum corrosion of an acidic sulfate-chloride nickel electrolyte such as described in my aforementioned application is reached at a sodium chloride content of approximately 30 grams per liter. Addition of chlorides in excess of this amount or conversion to all-chloride solutions of equal chloride concentrations does not increase the corrosive action of the acidic solution. The terms, "sulfate-chloride" and "all-chloride," employed herein, refer to the predominant negatively-charged ions in the aqueous solution. Sulfate-chloride solutions are those solutions containing substantial amounts of sulfate ions in addition to chloride ions whereas all-chloride solutions are substantially devoid of sulfate ions. Of course, the solutions may also contain small amounts of buffers, brighteners, corroding agents, or other addition agents or modifiers.

While the compositions contemplated by the present invention are particularly suitable for use with the highly corrosive solutions described hereinbefore, it is to be understood that the invention is applicable generally to corrosive acidic chloride-bearing aqueous solutions, particularly corrosive acidic sulfate-chloride or all-chloride aqueous solutions, and especially impure acidic solutions. To demonstrate the high corrosion resistance obtained by the present invention, it has been illustrated by reference to data obtained in particularly corrosive solutions.

Although the present invention has been described in conjunction with preferred embodiments, it is to be understood that modifications and variations may be resorted to without departing from the spirit and scope of the invention, as those skilled in the art will readily understand. Such modifications and variations are considered to be within the purview and scope of the appended claims.

I claim:

1. A cast corrosion resistant metal article containing 22% to 23% nickel, 21% to 22% chromium, 5% to 6% molybdenum, not exceeding 0.15% carbon and the balance essentially iron, and having an austenitic structure devoid of a sigma phase and of precipitated carbides at the grain boundaries, said article being in a condition resulting from an annealing treatment at about 2250° F. followed by rapid cooling.

2. A cast corrosion resistant metal article containing 21% to 23% nickel, 21% to 22% chromium, 5% to 6% molybdenum, not exceeding 0.15% carbon and the balance essentially iron, and having an austenitic structure devoid of a sigma phase and of precipitated carbides at the grain boundaries, said article being in a condition resulting from an annealing treatment at about 2250° F. followed by quenching.

3. A cast corrosion resistant metal article comprised of an annealed and quenched alloy containing 22% to 23% nickel, 21% to 22% chromium, 5% to 6% molybdenum, not exceeding 0.15% carbon and the balance essentially iron, and having an austenitic structure substantially devoid of a sigma phase and of precipitated carbides at the grain boundaries.

4. A cast corrosion resistant metal article comprised of an annealed and rapidly-cooled alloy containing 21% to 23% nickel, 21% to 22% chromium, the nickel content being at least as large as the chromium content, 5% to 6% molybdenum, not exceeding 0.15% carbon and the balance essentially iron, and having an austenitic structure devoid of a sigma phase.

5. A corrosion resistant metal article comprised of an alloy containing 21% to 23% nickel, 21% to 22% chromium, 5% to 6% molybdenum, not exceeding 0.15% carbon and the balance essentially iron, said alloy having an austenitic structure substantially devoid of a sigma phase and of precipitated carbides at the grain boundaries and being in a condition resulting from an annealing treatment at approximately 2250° F. followed by rapid cooling.

6. Chemical equipment subjected in use to contact with a corrosive acidic chloride-bearing aqueous solution comprised of a cast alloy containing 21% to 23% nickel, 21% to 22% chromium, 5% to 6% molybdenum, not exceeding 0.15% carbon and the balance essentially iron, said alloy having an austenitic structure substan-

tially devoid of a sigma phase and of precipitated carbides at the grain boundaries and being in a condition resulting from an annealing treatment at about 2250° F. followed by rapid cooling.

5 7. Chemical equipment subjected in use to contact with a corrosive acidic chloride-bearing aqueous solution comprised of an annealed and rapidly-cooled alloy containing 22% to 23% nickel, 21% to 22% chromium, 5% to 6% molybdenum, not exceeding 0.15% carbon and the balance essentially iron, and having an austenitic structure devoid of a sigma phase.

15 8. Chemical equipment subjected in use to contact with a corrosive acidic chloride-bearing aqueous solution comprised of an alloy having an austenitic structure devoid of a sigma phase and precipitated carbides at the grain boundaries and containing chromium within the range of 21% to 22% chromium, nickel in an amount at least equal to the chromium content and within the range of 21% to 23%, molybdenum within the range of 5% to 6%, not exceeding 0.15% carbon and the balance essentially iron, said alloy being in a condition resulting from an annealing treatment at about 2250° F. followed by quenching.

20 9. An alloy having a single-phase austenitic structure and comprised of 22% to 23% nickel, 21% to 22% chromium, 5% to 6% molybdenum, not exceeding 0.15% carbon and the balance essentially iron.

25 10. An alloy having an austenitic structure devoid of a sigma phase and comprised of 21% to 23% nickel, 21% to 22% chromium, 5% to 6% molybdenum, not exceeding 0.15% carbon and the balance essentially iron.

30 11. An alloy having an austenitic structure devoid of a sigma phase and comprised of chromium within the range of 21% to 22%, nickel in an amount at least equal to the chromium content and within the range of 21% to 23%, molybdenum within the range of 5% to 6%, not exceeding 0.15% carbon and the balance essentially iron.

LOUIS SECONDO RENZONI.

#### REFERENCES CITED

The following references are of record in the file of this patent:

#### FOREIGN PATENTS

|           |               |              |
|-----------|---------------|--------------|
| 50 Number | Country       | Date         |
| 508,710   | Great Britain | July 5, 1939 |

#### OTHER REFERENCES

55 The Effect of Molybdenum and Columbium on the Structure, Physical Properties and Corrosion Resistance of Austenitic Steels; pages 32 to 36 inclusive; Paper presented at the 22nd Annual Convention of the American Society for Metals, Cleveland, Ohio; October 20 to 25, 1940; by 60 Franks, Binder and Bishop, Electro-Metallurgical Co.